

## UNITED STATES PATENT OFFICE

2,262,970

## THERMOPLASTIC BOX TOES

Hymen Shrager and Barney Shinberg, Lawrence, Mass., assignors to Atlas Shoe Products Corporation, Lowell, Mass., a corporation of Massachusetts

No Drawing. Application February 12, 1938,  
Serial No. 190,325. Renewed January 16, 1940

7 Claims. (Cl. 36—77)

This invention relates to thermoplastic compositions for use in the manufacture of box toes for shoes.

In the manufacture of thermoplastic box toes, a sheet of suitable fibrous material such as steamed felt or water-laid felt is saturated with, in a hot bath, a thermoplastic composition, cooled, and then cut into blanks which are incorporated in the shoe structure, and the present invention is concerned primarily with the preparation of the thermoplastic composition.

The present invention has for its primary object to provide a thermoplastic composition which, when used as a saturant for fibrous material from which the shoe box toes are cut, will give a box toe blank having stiffness which will maintain the finished box toe in the desired shaped form with a sufficient flexibility to prevent distortion without cracking or breaking, and acquiring a tackiness when subjected to the steam of the lasting operation which causes a fusion of the toe cap to the lining and upper of the shoe without bleeding through and discoloring the lining or the shoe upper.

In the preparation of the composition embodying the present invention, rubber and copal are mixed together in a rubber mill with about five parts by weight of copal to four parts of rubber. Although there is in this mixture more copal than rubber, no difficulty of sticking is encountered on the rolls and the mixture can be milled and sheeted with very little trouble.

We prefer to use the grades of copal known as Manila CBB and Manila DBB, which grades consist of mixtures of Boea and Loba copals. These consist of small chips and nubs containing bark and other foreign material. The copal is given a preparatory treatment by grinding it and screening it through a 40 mesh screen. The copal-rubber mixture is then readily and uniformly blended.

The rubber-copal mixture is then dissolved in hot rosin or a mixture of rosin and Montan wax, or other suitable hard wax, a sufficient amount of the rubber-copal mixture being used to make the rubber in the total or final mixture amount to approximately 7%. Rubber added to the rosin or rosin wax mixture in this manner dissolves readily. The temperature required is not excessive and will not cause thermal decomposition of the rosin or the depolymerization of the rubber.

After preparing the composition in this manner, the fibrous material is then saturated therewith by dipping the material in a hot solution of the composition, and after the stock sheet thus

prepared has cooled, it may be cut into the desired box toe blanks.

The blanks prepared with the composition herein set forth are characterized by having a stiffness which causes them to maintain their proper shape when incorporated in a shoe structure but they are sufficiently resilient or flexible to permit slight deformation without becoming cracked or broken, and they are characterized further by becoming slightly tacky when subjected to the steam of the lasting operation so that the toe cap becomes fused to the lining and upper of the shoe without bleeding through or discoloring the lining or the shoe upper.

We are aware that other thermoplastics have been made for use in the manufacture of box toes which use rubber, but these compositions have disadvantages which are not present in the composition herein set forth.

20 In one such composition of which we are aware, vulcanized rubber is added directly to a rosin mixture, which procedure must lead to depolymerization of the rubber. By "rosin mixture" we refer to rosin and asphalt, or rosin along with the waxes or plasticizers commonly used in the manufacture of box toes. An alternative method of preparing this composition is by dissolving vulcanized rubber in a volatile solvent or by using a vulcanized latex and adding 25 these to the rosin mixture, resulting in compositions of inferior quality to the composition embodying the present invention. In the procedure set forth in this application, the rubber-copal mixture swells immediately on being added to the rosin and dissolves readily without depolymerization.

25 In another process known to us, rubber is milled with a protective colloid. When this is added to the rosin bath, a two-phase mixture is 30 formed, the particles of rubber being protected by a hydrophilic colloid, the rosin mixture forming the continuous phase of the dispersion. The mixture embodying the present invention is prepared without the use of a protective colloid and 35 is single phased.

The rubber used in the present mixture with the copal is in the form of a solidified rubber latex which is not given any particular treatment before being mixed with the copal other than the usual milling by which the rubber is broken down to a workable condition.

While it is preferred that the composition be prepared with rosin alone or with a mixture of rosin and Montan wax, it is possible to use other cheap resins with the rubber-copal mixture. For

example, cumar resin may be used or there may be used a mixture of wood rosin and Vinsol and the rubber-copal mixture dissolved in these resins. Vinsol is a hard, brittle thermoplastic material of resinous nature produced from the Southern long leaf pine. While a thoroughly satisfactory mixture is obtainable by mixing the rubber-copal mixture with these other resins, the best results are obtained with rosin alone or a mixture of rosin and Montan wax. Carnauba wax may also be employed in place of the Montan wax.

As an example of a composition using rosin and wax, a mixture of six parts wood rosin and one part Montan wax may be made, and in this may be dissolved the previously referred rubber-copal mixture made up in the proportions respectively of 4 to 5. In this mixture the rubber-copal combination will be employed in a quantity sufficient to make the rubber content approximate 7% of the entire mass.

What we claim is:

1. The improved thermoplastic box toe having a body of fibrous material permeated with a composition comprising essentially rosin, and a minor quantity of a mixture of copal and rubber, in which the rubber constitutes approximately seven percent of the composition and the box toe being characterized in that it acquires a tackiness when subjected to the steam of a lasting operation which effects its fusion to adjacent elements of the shoe structure into which it is built.

2. The improved shoe box toe stock consisting of a body of sheet material impregnated with a mixture of rosin and hard wax combined in the proportions, respectively, of six to one, and a mixture of rubber and copal which are in the proportions, respectively, of four to five, the said rubber copal mixture being incorporated in the

stock in an amount sufficient to make the rubber content approximately 7% of the entire impregnated material.

3. The improved box toe stock having a base or carrier body of fibrous material impregnated with a composition comprising essentially rosin having a minor quantity of a milled mixture of rubber and copal dissolved therein, in which the rubber content of the mixture is approximately 7%.

4. The improved box toe stock having a base impregnated with a composition comprising essentially rosin and a minor quantity of a milled mixture of rubber and copal dispersed in the rosin, in which the rosin content of the mixture is approximately 73%.

5. The improved box toe stock consisting of a base impregnated with a composition consisting of a rosin and wax mixture combined with and having dissolved therein a milled mixture of rubber and copal, the rosin and wax being in the proportions respectively of six to one.

6. The improved box toe stock consisting of a base impregnated with a composition consisting of a rosin and wax mixture combined with and having dissolved therein a milled mixture of rubber and copal, the rosin and wax being in the proportions respectively of six to one and the rubber and copal being in the proportions respectively of four to five.

7. The improved box toe stock consisting of a base impregnated with a composition consisting of a rosin and wax mixture combined with and having dissolved therein a milled mixture of rubber and copal, and the two mixtures being proportioned in the composition to give to the box toe a rubber content of approximately 7%.

HYMEN SHRAGER.  
BARNEY SHINBERG.